

March 25, 1930.

D. M. FLOURNOY ET AL

1,752,164

PROCESS FOR ORNAMENTING SURFACES

Filed July 28, 1927



INVENTORS

D. M. FLOURNOY

P. D. GEORGE

BY

*S. C. Stagg*  
ATTORNEY

## UNITED STATES PATENT OFFICE

DAVID M. FLOURNOY AND PERICLES D. GEORGE, OF ST. LOUIS, MISSOURI

## PROCESS FOR ORNAMENTING SURFACES

Application filed July 28, 1927. Serial No. 209,133.

Our invention relates to a process for ornamenting surfaces, one particular application of the process being the manufacture of coated material for use in making water proof garments, coverings, and the like. Water proof textile material heretofore used, for example, in the manufacture of rain proof garments, has either had a rough, unattractive surface or a smooth surface without pattern or design. In accordance with our invention or discovery we are enabled to make an ornamented water proof material by a process little if any more expensive than those heretofore employed in the manufacture of plain, smooth material.

In its application to the manufacture of material for rain proof garments, our process comprises impregnating a woven fabric, preferably silk, with a liquid material, which when coagulated or "dried" in a film is flexible; viscous linseed oil being an example of such liquid. Other drying oils such as soya bean oil, or Perilla oil may be used, either alone or mixed with linseed oil, as the impregnating liquid. In application this treatment comprises immersing the fabric in the liquid and then passing it between rollers, or other known means, to remove the surplus liquid and predetermine the thickness of the product before drying. The treated fabric is then dried, preferably by application of heat, and the resultant product is a flexible sheet having the combined strength of the film and the fabric and impervious to water; but its surfaces are without figure or pattern and it is not of attractive appearance in a manufactured garment. In order to give the product an attractive appearance, and incidentally further increasing the thickness of water proof material without, however, substantially affecting the flexibility, we apply to it a coating of a liquid composition consisting of two parts viscous linseed oil and one part of China wood oil, preferably with the addition of a drier in the form of linoleate of lead, cobalt, or manganese, and also preferably with approximately 15% by volume of a suitable thinner, such as petroleum naphtha. It is known that when viscous China wood oil, (produced by heat treating

the raw oil) coagulates after being spread as a coating, it forms a wrinkled surface and that the cross sectional dimensions of the wrinkles varies somewhat with varying viscosity of the oil. Prior to our invention, however, this characteristic of China wood oil has had little, if any, practical value on account of lack of knowledge as to how to control the effect, nor had it been conceived that it could be employed to produce an ornamental surface on a fabric. The China wood oil used in the composition above described is heat treated to give it such viscosity as to give the composition the characteristic that when employed as a coating and treated as hereinafter described, it coagulates in drying to produce a uniform wrinkled surface comprising small ridges or "wrinkles" closely adjacent to each other. The degree of viscosity of the oil necessary that the composition have the characteristic referred to, is not critical and a suitable degree may readily be obtained by test in carrying out our improved process. In the claims we have employed the word "treated" to define China wood oil having suitable viscosity for the purposes of our invention.

The final coating just described, is applied to the product resulting from the first portion of the process above described, one suitable means for so applying it being to immerse the product in the composition, then pass it between rolls, or other known means, to determine the thickness of the applied film. A suitable thickness to accomplish the desired result may readily be determined by experiment, it being noted here that it is possible to make this film both too thin and too thick to secure the preferred ornamental appearance hereinafter described, or any definite uniform pattern over all of the treated material. Promptly after applying to the material the second coating referred to, it is passed into an oven and subjected to a temperature of not less than 110° F. We have found that in a few minutes after being subjected to heat the outer film coagulates in tiny ridges in close proximity to each other and over the entire surface, there being areas of substantially parallel ridges, other areas in

which the ridges are in fan shape, and areas in which they are irregular. The accompanying drawing is intended to illustrate approximately the lining of the surface as just described. It is characteristic that the entire surface presents the desired ornamental effect, and that the lines or ridges are substantially uniform in height and width. The silk being translucent, and the films resulting from the drying of both of the treating materials being transparent or translucent, the light transmission and reflection combines with the physical conformation of the surface to produce a very pleasing visual effect.

15 It will be noted that the process described does not involve any materials or treatment injurious to the base fabric or the application of any chemical reagents to the films in either their liquid or coagulated state.

20 While we do not desire to be bound to any theory or explanation of the causes of the forming of the particular surface resulting from our process, we believe that it is partly due to the adjustment of thickness of the second film and the immediate application of the proper degree of heat thereto, since we have found that the film will not produce the ornamental effect if the application of heat is delayed very long. This would indicate a particular range of thicknesses of the second film applied and the prompt application of heat is what causes it to regularly form in fine lines or ridges of uniform size distributed entirely over the surface and thus makes the process useful by reason of the controllability of the ornamental result. The desired ornamental appearance would not be secured on a silk fabric by omitting the first treatment herein described from which it appears to be essential that the surface to which the China wood oil composition is applied to be fairly smooth, or at least have more resistance to contraction than the silk fabric itself.

45 It will be understood that we do not intend that our invention be limited to the use of the particular substances herein described. Such other materials as may have similar characteristics to treated China wood oil with respect to the surface of a coagulated film thereof would of course be the equivalent of China wood oil for the broader purposes of our invention; likewise, since the result broadly desired from the employment of the second coating is a flexible wrinkled film and the wrinkling effect is produced by the China wood oil, the other coagulable oil used with it to form the second coating, may, in lieu of linseed oil be Perilla oil or other coagulable oils which may be caused to dry at a suitable rate and will give the dried film the suitable flexibility which it would not have if the second coating were composed solely or chiefly of China wood oil.

Having fully described our invention,

what we claim as new and desire to secure by Letters Patent of the United States is:

1. The process of producing an ornamental water proof cloth, which comprises impregnating woven silk fabric with a liquid composition coagulable to form a flexible water proof material and applying to said product after the composition has been coagulated, a coating of a coagulable mixture containing treated China wood oil and promptly subjecting said coating to heat. 75

2. The process of forming an ornamental water proof material adapted for use in coverings, wearing apparel, and the like, which comprises immersing silk fabric in a liquid compound capable of forming a flexible film when dried, passing the treated fabric through rolls, or other known means, to remove the surplus liquid, drying the same, and then applying to the surface thereof a coating of a coagulable liquid composition containing China wood oil and promptly subjecting the material to heat to quickly coagulate the mixture, the China wood oil of the composition being of such viscosity as to cause the surface of the coating to contract in drying under said prompt application of heat to form a pattern whose dominating characteristic is a plurality of closely adjacent ridges of substantially uniform cross sectional area and uniformly distributed over the entire surface. 80 90

3. The process of forming an ornamental water proof material adapted to use in coverings, wearing apparel, and the like, which comprises immersing silk fabric in a liquid compound capable of forming a flexible film when dried, passing the treated fabric through rolls, or other known means, to remove the surplus liquid, drying the same, and then applying to the surface thereof a coating of a mixture of one part treated China wood oil and two parts linseed oil, said mixture also containing linoleate of lead, or an equivalent drier, and petroleum naphtha, or equivalent thinner, and promptly subjecting the material to atmospheric air of a temperature of at least 110° F. 100 110

4. The process of ornamenting a fabric which comprises applying thereto a coating of a liquid capable of forming a smooth film when dried, applying to said coating when dry a coagulable liquid mixture comprising treated China wood oil and having the characteristic of such surface contraction in coagulating in heated atmospheric air as to form a ridged surface, and promptly subjecting said applied coating to heat. 115 120

5. The process of forming ornamental water proof material adapted to use in coverings, wearing apparel and the like, which comprises immersing silk fabric in viscous linseed oil, removing the surplus liquid therefrom, drying the same, and then applying to the surface of said dried coating a 125 130

coagulable oil composition comprising treated China wood oil, and promptly subjecting the material to atmospheric air of a temperature of at least 110 degrees F.

5 In testimony whereof, we hereunto affix our signatures, this 25 day of July, 1927.

DAVID M. FLOURNOY.  
PERICLES D. GEORGE.

10

15

20

25

30

35

40

45

50